

## [54] ELECTROPHOTOGRAPHIC RECORDING MATERIAL

[75] Inventor: Wolfgang Wiedemann,  
Geisenheim-Johannisberg, Germany[73] Assignee: Kalle Aktiengesellschaft,  
Wiesbaden-Biebrich, Germany

[22] Filed: Apr. 25, 1973

[21] Appl. No.: 354,201

## [30] Foreign Application Priority Data

July 31, 1972 Germany ..... 2237680

[52] U.S. Cl. .... 96/1.5, 96/1.6

[51] Int. Cl. .... G03g 5/06

[58] Field of Search ..... 96/1.5, 1.6

## [56] References Cited

## UNITED STATES PATENTS

3,573,906 4/1971 Goffe ..... 96/1.5

Primary Examiner—Ronald H. Smith

Assistant Examiner—J. P. Brammer

Attorney, Agent, or Firm—James E. Bryan, Esq.

## [57] ABSTRACT

This invention relates to an electrophotographic recording material consisting of an electroconductive support material and a photoconductive double layer of organic materials which consists of a homogeneous, opaque, charge carrier producing dyestuff layer from a compound of the general formula



in which X<sub>1</sub> and X<sub>2</sub> are identical or different and stand for —NH— or —S— and Ar and Ar' may be substituted, such compounds being particularly suitable as are substituted in peri position to the —C=O, —S— or —NH—group in the five-membered ring and of a transparent top layer of insulating materials with at least one charge transporting compound.

16 Claims, 3 Drawing Figures



PATENTED OCT 1 1974

3,839,034

SHEET 1 OF 6



Fig. 1



Fig. 2



## FORMULAE

1



2



3



4



5



## FORMULAE

6



7



8



9



10



## FORMULAE

11



12



13



14



15



PATENTED OCT 1 1974

3,839,034

SHEET 6 OF 6

## FORMULAE



## ELECTROPHOTOGRAPHIC RECORDING MATERIAL

This invention relates to an electrophotographic recording material consisting of an electroconductive support material and a photoconductive double layer of organic materials which consists of a homogeneous, opaque, charge carrier producing dyestuff layer from a compound of the general formula



in which  $X_1$  and  $X_2$  are identical or different and stand for  $-\text{NH}-$  or  $-\text{S}-$  and  $\text{Ar}$  and  $\text{Ar}'$  may be substituted, such compounds being particularly suitable as are substituted in peri position to the  $=\text{C}=\text{O}$ ,  $-\text{S}-$  or  $-\text{NH}-$  group in the five-membered ring and of a transparent top layer of insulating materials with at least one charge transporting compound.

It is known from German Offenlegungsschriften Nos. 1,597,877 and 1,797,342 for electrophotographic recording material to extend the spectral sensitivity of selenium layers to the red spectral range by a double layer arrangement, e.g., with phthalocyanine dispersion layers. Disadvantageous are the vacuum vapor depositions of selenium requiring high technical expenditure, the brittleness of comparatively thick selenium layers, the poor adhesion of adjacent heterogeneous constituents in these layers and the only difficulty realizable uniformly wetting coating with the corresponding dispersions. Furthermore, no optimum light-sensitivities can be achieved as a result of the absorption behaviour and the different charge conducting mechanisms of selenium and phthalocyanine in the double layer arrangement.

From U.S. Pat. No. 3,573,906, for example, there are also known photoconductive double layers containing an organic, possibly photoconductive, insulating layer between the support material and the vapor-deposited selenium layer in order to impart adhesion. Such a layer construction, however, considerably hinders the necessary charge transport so that, in this case too, no higher light-sensitivities are obtainable.

Furthermore, from German Auslegeschrift No. 1,964,817, it is known to provide vapor-deposited selenium layers with a layer of an organic, photoconductive insulating material which is substantially insensitive to light in the visible range of the spectrum. According to German Offenlegungsschrift No. 2,120,912, it has also been suggested to use those light-sensitive layer arrangements for electrophotographic recording materials which contain, as the charge carrier producing layer, an inorganic material, such as the sulfide, selenide, sulfoselenide or telluride of cadmium or zinc, and as the charge carrier transporting layer, an organic material with at least 20 per cent by weight of 2,4,7-trinitro-9-fluorenone. A disadvantage of the production of these layers with inorganic photoconductors is the exact observation of the vapor deposition conditions of selenium or the exact adjustment of the mixtures in order to obtain a good photoconductive modification of the inorganic materials. Furthermore, the adhesion of selenium to conductive support material, such as to

aluminum, is insufficient. Fatigue in repeated charge/exposure cycles does not allow the use in electrophotographic copying devices.

Japanese Patent Application No. 43-26710 already discloses photoconductive double layers of organic materials on a conductive support. According to that application, a lower, relatively thick layer of a considerably diluted homogeneous solution of a sensitizer in a binder is provided with an upper transparent light-sensitive layer. This layer construction, however, only offers a relatively low sensitivity increase only little meeting technical demands. Another known suggestion according to German Offenlegungsschrift No. 1,909,742 is to repeatedly pour a sensitizer solution over a photoconductive layer and to evaporate the solvent. A disadvantage thereof is the low mechanical resistance of the applied layer as a result of insufficient cohesion and adhesion of the applied sensitizer. Furthermore, repeated coating is cumbersome.

The construction of photoconductive double layers containing a dyestuff layer is also known, e.g. from Belgian Patents Nos. 763,389 and 763,541, but for this layer construction, top layers are used which allow no sensitivities satisfying highest demands and, as regards adhesion between the dyestuff layer and the top layer, do not represent an optimization and are not sufficiently resistant to mechanical attack, e.g., in electrophotographic copying devices, particularly to that due to the cleaning of the photoconductive layer.

It is the object of the present invention to provide an organic photoconductor layer highly light-sensitive for the xerographic copying procedure which overcomes the described disadvantages and the adhesion of which between the various layers satisfies the highest technical demands, which exhibits no wear or fatigue and which, even after repeated use, may be used again rapidly.

The present invention provides an electrophotographic recording material consisting of an electroconductive support material with a photoconductive double layer of organic materials which consists of a homogeneous, opaque, charge carrier producing dyestuff layer from a compound of the general formula



in which  $X_1$  and  $X_2$  are identical or different and stand for  $-\text{NH}-$  or  $-\text{S}-$  and  $\text{Ar}$  and  $\text{Ar}'$  may be substituted, such compounds being particularly suitable as are substituted in peri position to the  $=\text{C}=\text{O}$ ,  $-\text{S}-$  or  $-\text{NH}-$  group in the five membered ring and of a transparent top layer of insulating materials with at least one charge transporting compound and is characterized in that the transparent top layer consists of a charge transporting, monomer, heterocyclic compound substituted by at least one dialkyl amino group or two alkoxy groups and having an extended  $\pi$ -electron system or of a condensation product from 3-bromopyrene and formaldehyde and of a binder.

By means of the invention, it is possible to obtain highly light-sensitive, photoconductive double layers for the electrophotographic recording material of the invention which have a high mechanical resistance and

may be arranged on a cylindrical drum, for example, or may circulate as an endless belt without exhibiting special signs of wear and thus are very suitable for the use in electrophotographic copying devices. The high light-sensitivity particularly results from the fact that the charge transporting compound present in the transparent top layer is sensitized by the charge carrier producing dyestuff layer in that the charge carriers, such as electrons or holes are taken by the top layer.

In a preferred embodiment, the organic dyestuff layer has a thickness in the range from about 0.005 to about 2  $\mu\text{m}$ . High concentration of excited dyestuff molecules is achieved thereby in the dyestuff layer and at the boundary surface between the dyestuff layer and the top layer. It has proved that layer thicknesses from about 0.005 to about 1  $\mu\text{m}$  are entirely sufficient and that even layers in the range of about 0.001  $\mu\text{m}$  may be effective. Furthermore, the adhesion between the electroconductive support material and the top layer is not impaired.

In a preferred embodiment, the transparent top layers has a thickness in the range from about 5 to about 20  $\mu\text{m}$ . This assures a sufficiently high charge.

The assembly of the electrophotographic recording material can be seen in the attached FIGS. 1 and 2. FIG. 1 shows a material which consists of an electroconductive layer support 1, the organic dyestuff layer 2, and the organic, transparent top layer 3. FIG. 2 shows a metallized plastic layer 1, 4 as the layer support to which a charge carrier injection inhibiting intermediate layer 5 is applied and the photoconductive double layer from organic dyestuff layer 2 and organic, transparent top layer 3 is on this intermediate layer.

Suitable electroconductive support materials are materials which hitherto have been used for this purpose, for example aluminum foils or transparent plastic supports to which aluminum, gold, copper, zinc, cadmium, indium, antimony, bismuth, tin, lead or nickel has been laminated or applied by vapor deposition.

As shown in FIG. 2, an organic intermediate layer or a thermally, anodically or chemically produced metal oxide layer, e.g., aluminum oxide layer, may be applied to the electroconductive support material. This layer serves to decrease or to prevent charge carrier injection in the dark from the electroconductive support material into the organic dyestuff layer. On the other hand, it may not hinder, however, the flowing off of charge during exposure to light. Furthermore, the intermediate layer provides for a favorable influence of the adhesion of the organic dyestuff or double layer to the support material. Suitable as organic intermediate layers are various natural or synthetic resin binders which firmly adhere to a metal or aluminum surface and, upon subsequent application of the other layers, are not dissolved. Polyamide resins or polyvinyl phosphoric acid are particularly suitable for this purpose.

The thickness of the organic intermediate layer is in the range of about 1  $\mu\text{m}$ , that of a metal oxide layer in the range from  $10^2$  to  $10^4$  angstroms.

The organic dyestuff layer of the recording material of the invention substantially determines the spectral light-sensitivity of the photoconductive double layer of the invention. The dyestuffs used are known compounds described in the Color Index, 2nd edition (1956), volume 3. Such dyestuffs are, for example, those listed in the attached formula table.

The meanings are as follows:

| Formula No. | Name                                   | C.I.   |
|-------------|----------------------------------------|--------|
| 1           | Indigo                                 | 73,000 |
| 2           | Thioindigo; Algol Red 5B               | 73,300 |
| 3           | Indanthren Printing Red 3B             | 73,305 |
| 4           | Indanthren Brilliant Pink R            | 73,360 |
| 5           | Indanthren Red Violet RH               | 73,385 |
| 6           | Indazin Bordeaux RRL                   | 73,395 |
| 7           | Permanent Red Violet MR Pigment Red 88 |        |
| 8           | Algol Orange RF                        | 73,335 |
| 9           | Indanthren Brilliant Pink 3B           | 73,365 |
| 10          | Indanthren Scarlet B                   | 73,355 |
| 11          | Vat Violet RR                          | 73,600 |
| 12          | Algol Violet BBN                       | 73,605 |
| 13          | Indanthren Printing Violet BBF         | 73,595 |
| 14          | Indanthren Printing Brown R            | 73,665 |
| 15          | Indanthren Brown RRD                   | 73,410 |
| 16          | Brilliant Indigo B                     | 73,040 |
| 17          | Brilliant Indigo 4B                    | 73,065 |

20 The organic dyestuff layer must be extremely uniform since only its uniformity guarantees a uniform injection of charge carriers into the top layer.

To achieve this object, the dyestuff layers are applied according to special coating methods. Such methods are the application by mechanically rubbing the most finely powdered dyestuff material into the electroconductive support material, the application by chemical deposition of a leucobase to be oxidized, for example, the application by electrolytical or electrochemical processes or the gun spray method. The application preferably is performed, however, by vapor depositing the dyestuff in the vacuum. A tightly packed coating is achieved thereby.

35 The tightly packed coating makes it unnecessary to produce thick dyestuff layers for achieving a high absorption.

The tightly packed dyestuff molecules and the extremely low layer thickness permit, in a particularly advantageous manner, the transport of charge carriers so that it is completely sufficient to produce the charge carriers at the boundary layer only.

40 The application of the dyestuff layer by vapor deposition in the vacuum requires dyestuffs with thermal resistivity in the temperature range to be applied for vapor deposition. The high extinction of the dyestuff allows high concentration of excited dyestuff molecules. Excitation (1) and charge separation (2) take place in the dyestuff layer according to the following reaction equations:



55  $S$  - dyestuff molecule

60  $S^*$  - excited dyestuff molecule, and

$\cdot S^+, \cdot S^-$  - dyestuff radical ions.

At the boundary surface between the organic dyestuff layer and the transparent top layer, reactions of the excited dyestuff molecules or the resulting charge carriers in the form of the dyestuff radical ions with the molecules of the charge transfer effecting compound in the top layer are possible according to the following equations:

3.  $S^* + F_1 \rightarrow \cdot S^- + \cdot F_1^+$
4.  $S^* + F_2 \rightarrow \cdot S^+ + \cdot F_2^-$
5.  $\cdot S^+ + F_1 \rightarrow S + \cdot F_1^+$
6.  $\cdot S^- + F_2 \rightarrow S + \cdot F_2^-$

with

$F_1$  - donor molecule

$F_2$  - acceptor molecule

$\cdot F_1^+$ ,  $\cdot F_2^-$  - donor or acceptor radical ion

At the boundary surface, sensitizing reactions take place between the transparent top layer and the organic dyestuff layer. The top layer thus is a sensitized organic photoconductor at least in the area of the boundary surface, which leads to the surprisingly high 15 photoconductivity.

Reactions 3 and 5 proceed preferably when the  $\pi$ -electron system in the top layer is a compound which, as a donor compound, easily can release electrons. This is the case with 2,5-bis-(4-diethylaminophenyl)-oxiazole-1,3,4, for example. But also heterocyclic compounds with only one dialkyl amino group are suitable for rapid procedure of reactions 3 and 5. Reactions 4 and 6 are preferably possible with a substance in the top layer which, as an electron acceptor easily accepts electrons, e.g. 2,4,7-trinitrofluorenone or 3,6-dinitro-N-t-butyl-naphthalimide.

By means of the specific embodiment of the invention it is sufficient for the efficiency of the dyestuff when, besides its intense absorption, it only has either electron-attracting substituents, e.g.  $> C = O$ ,  $-NO_2$ , halogen, or electron-repelling substituents, e.g. alkyl or O-alkyl, depending on whether it is preferably suitable for reactions 3, 5 or 4, 6.

The invention permits charge carrier transport fostered by a particularly low expenditure of energy within the tightly packed dyestuff layer according to the following reactions:



In all conventional sensitizing processes, however, transport via the dyestuff molecules present in low concentration is impeded by their large distance from one another. Analogous is the charge transport in the top layer with:



The practical consequence of reactions 1 to 10 is that, in the use of electron donors in the top layer, the double layer arrangement is negatively charged so that reactions 3, 5, 8, 9 can proceed. In the inverse case, layers with electron acceptors in the top layer are positively charged so that reactions 4, 6, 7 and 10 can proceed.

The transparent top layer or organic insulating materials with at least one charge transporting compound is described as follows:

The transparent top layer has a high electric resistance and prevents in the dark the flowing off of the electrostatic charge. Upon exposure to light, it transports the charges produced in the organic dyestuff layer.

In the case of negative charge, the transparent top layer preferably consists of a mixture of an electron

donor compound and a binder. But when the electro-photographic recording material is to be used for positive charge the transparent top layer consists of a mixture of an electron acceptor compound and a binder.

5

Consequently, in the transparent top layer there are used compounds for charge transport which are known as electron donors or electron acceptors. They are used together with binders or adhesives adapted to the compound for charge transport as regards charge transport, film property, adhesion, and surface characteristics. Furthermore, conventional sensitizers or substances forming charge transfer complexes are preferably additionally present. But they can only be used in so far as the necessary transparency of the top layer is not impaired. Finally, other usual additives such as levelling agents, plasticizers, and adhesives may also be present.

20 Suitable compounds for charge transport are especially those organic compounds which have an extended  $\pi$ -electron system, e.g., monomer aromatic heterocyclic compounds.

Monomers employed in accordance with the invention are those which have at least one dialkyl amino group or two alkoxy groups. Particularly proved have heterocyclic compounds, such as oxiazole derivatives, which are mentioned in German Patent No. 1,058,836. An example thereof is in particular the 2,5-bis-(p-diethylaminophenyl)-oxiazole-1,3,4. Further suitable monomer electron donor compounds are, for example, triphenyl amine derivatives, benzo-condensed heterocycles, pyrazoline or imidazole derivatives, as well as triazole and oxazole derivatives, e.g. 2-phenyl-4-(2-chlorophenyl)-5-(4-diethylaminophenyl)-oxazole, as disclosed in German Patents Nos. 1,060,260, and 1,120,875. Formaldehyde condensation products with various aromates, e.g., condensates from formaldehyde and 3-bromopyrene, are also suitable.

40 Besides these mentioned compounds having predominantly a p-conductive character, it is also possible to use n-conductive compounds. These so-called electron acceptors are known from German Patent No. 1,127,218, for example. Compounds such as 2,4,7-trinitrofluorenone or N-t-butyl-3,6-dinitro-naphthalimide have proved particularly suitable.

45 Suitable binders with regard to flexibility, film properties, and adhesion are natural and synthetic resins. Examples thereof are in particular polyester resins, e.g., those marketed under the names Dynapol (Dynamit Nobel), Vitel (Goodyear), and which are copolymers of iso- and terephthalic acid with glycol. Silicone resins are those known under the name SR of General Electric Comp., USA, or Dow 804 of Dow Corning Corp., USA, and representing three-dimensionally cross-linked phenyl-methyl siloxanes or so-called reactive resins as those known as DD lacquers and composed of an equivalent mixture of hydroxyl groups containing polyesters or polyethers and polyfunctional isocyanates, e.g. Desmophen and Desmodur of Bayer AG, Leverkusen, Germany, have proved particularly suitable. Furthermore, copolymers of styrene and maleic acid anhydride, e.g. those known under the name Lytron (R), Monsanto Chemical Comp., USA, but also polycarbonate resins, e.g. those known under the name Lexan Grade (R) of General Electric Comp., USA, are suitable for use.

50 55 60 65

The mixing ratio of charge transporting compound to binder may vary. Relatively certain limits are given, however, by the requirement for maximum photosensitivity, i.e., for the biggest possible portion of charge transporting compound, and for crystallization to be prevented, i.e., for the biggest possible portion of binder. A mixing ratio of about 1:1 parts by weight has proved preferably, but mixing ratios from about 3:1 to 1:4 or above, depending on the particular case, are also suitable.

The conventional sensitizers to be used additionally may advantageously foster charge transport. Moreover, they may produce charge carriers in the transparent top layers. Suitable sensitizers are, for example, Rhodamine B extra, Schultz, Farbstofftabellen (dyestuff tables), 1st volume, 7th edition, 1931, No. 864, page 365, Brilliant Green, No. 760, page 314, Crystal Violet, No. 785, page 329, and Cryptocyanine, No. 927, page 397. In the same sense as act the sensitizers may also act added compounds which form charge transfer complexes with the charge transporting compound. Thus, it is possible to achieve another increase of the photosensitivity of the described double layers. The quantity of added sensitizer or of the compound forming the charge transfer complex is so determined that the resulting donor acceptor complex with its charge transfer band still is sufficiently transparent for the organic dyestuff layer below. Optimum concentration is at a molar donor/acceptor ratio of about 10:1 to about 100:1 and vice versa.

The addition of adhesives as binders to the charge transporting compounds already yields a good photosensitivity. In this case, low-molecular polyester resin, such as Adhesive 49 000, Du Pont, has proved particularly suitable.

In the described manner, the top layers have the property to render possible a high charge with a small dark discharge. Whereas in all conventional sensitizations an increase of the photosensitivity is connected with an increase of the dark current, the arrangement of the invention can prevent this parallelity. The layers are thus usable in electrophotographic copying devices with low copying speeds and very small lamp energies as well as in those with high copying speeds and correspondingly high lamp energies.

The top layers are prepared according to the usual coating methods, e.g., whirl-coating, doctoring, kiss-coating.

The invention will be further illustrated by way of the attached drawings.

#### Preparation of the dyestuff layers:

The dyestuffs listed in Table 1 are vapor deposited by a vacuum pump (Type A 1 of Pfeiffer, Wetzlar, Germany) at a reduced pressure of  $10^{-3}$  to  $10^{-4}$  mm Hg onto a  $100\mu\text{m}$  thick aluminum foil arranged at a distance of about 15 cm. The vapor deposition temperature is measured directly at the surface of the dyestuff to be vapor deposited by means of a NiCr-thermoelement. The layer weight of the vapor deposited dyestuff is in the range from about 0.01 to 1 g/m<sup>2</sup>.

Table 1

| Dyestuff                          | No. | Vapor deposition |                  |
|-----------------------------------|-----|------------------|------------------|
|                                   |     | Time (min)       | Temperature (°C) |
| Indigo                            | 1   | 0.5              | 180              |
| Thioindigo                        | 2   | 1                | 230              |
| Indanthren<br>Printing Red 3B     | 3   | 2                | 270              |
| Indanthren<br>Brilliant Pink R    | 4   | 2                | 270              |
| Indazin<br>Bordeaux RRL           | 6   | 2                | 230              |
| Permanent Red                     |     |                  |                  |
| Violet MR                         | 7   | 2                | 300              |
| Vat Violet RR                     | 11  | 1                | 230              |
| Indanthren<br>Printing Violet BBF | 13  | 1                | 270              |
| Indanthren Brown RRD              | 15  | 3                | 350              |

## Example 1

Homogeneous dyestuff layers, from thioindigo dyestuffs, which have been obtained by vapor deposition as described in Table 1 or under analogous conditions are coated with a solution from

1 part by weight of 2,5-bis-(4-diethylaminophenyl)-oxadiazole-1,3,4 and

1 part by weight of polyester resin, e.g. Dynapol L 206 of Dynamit Nobel AG, Troisdorf, Germany, in tetrahydrofuran as the solvent. After drying for 5 minutes at 120°C, the thickness of the top layer is about 9 to  $11\mu\text{m}$ .

The photosensitivities of these double layers are summarized in Table 2.

They are determined according to the following method: On a slowly rotating disk, the photoconductor layer moves through a charging device (corona adjustment 7.0 kV, grid 1.5 kV) to the exposure section where it is exposed to an Osram xenon lamp, type XBO

150 A heat absorbing glass, (type KG 3 of Schott & Gen., Mainz, Germany) and a neutral filter of 15 per cent transparency are placed before the lamp so that the light intensity in the plane of measurement is about  $750\mu\text{W}/\text{cm}^2$ . The charge height ( $U_0$ ) and the curve of

50 the photo-induced light decay are oscilloscopically recorded by an electrometer (type 610 CR of Keithley Instruments, USA) through a transparent probe. The determination of the charge height ( $U_0$ ) in volts and of the half time ( $T_{1/2}$ ) in milliseconds yields the following 55 results for the double layers as well as for a correspondingly prepared top layer without dyestuff (zero layer):

| No. | Double layer with dyestuff                  | Formula No. | $U_0(\text{V})$<br>Negative charge | $T_{1/2}$<br>(msec) | $\Delta U_0$ |
|-----|---------------------------------------------|-------------|------------------------------------|---------------------|--------------|
| 1   | zero layer                                  | —           | 900                                | 240                 | —            |
| 2   | Algol Red 5B/<br>top layer                  | 2           | 1,075                              | 124                 | 75           |
| 3   | Indanthren<br>Printing Red 3B/<br>top layer | 3           | 1,050                              | 98                  | 55           |

## -Continued

| No. | Double layer with dyestuff              | Formula No. | U <sub>o</sub> (V) Negative charge | T <sub>1/2</sub> (msec) | ΔU <sub>D</sub> | Double layer with dyestuff | Formula No.                               | U <sub>o</sub> (V) negative charge | T <sub>1/2</sub> (msec) |
|-----|-----------------------------------------|-------------|------------------------------------|-------------------------|-----------------|----------------------------|-------------------------------------------|------------------------------------|-------------------------|
| 4   | Indanthren Brilliant Pink R/ top layer  | 4           | 1,075                              | 16                      | 80              | 5                          | Formula No. 9                             | 875                                | 19                      |
| 5   | Indanthren Red Violet RH/ top layer     | 5           | 1,200                              | 22                      | 50              | 10                         | Indanthren Brilliant Pink R Formula No. 4 | 800                                | 31                      |
| 6   | Indanthren Brilliant Pink 3B/ top layer | 9           | 1,050                              | 12                      | 95              | 15                         |                                           |                                    |                         |
| 7   | Permanent Red Violet MR/ top layer      | 7           | 925                                | 16                      | 135             | 20                         |                                           |                                    |                         |
| 8   | Algol Orange RF/ top layer              | 8           | 900                                | 80                      | 70              |                            |                                           |                                    |                         |
| 9   | Indanthren Scarlet B/ top layer         | 10          | 1,075                              | 68                      | 70              |                            |                                           |                                    |                         |

The determination of the dark decay ( $\Delta U_D$ ) is important for the use of the photoconductor layers in xerographic copying machines. This value is thus included in Table 2. It shows how rapidly a photoconductor layer is discharged in the dark after period of 2 seconds, after it has achieved its maximum charge. The dark decay is measured by a Dyn-Test 90 apparatus of ECE, Giessen, Germany. The spectral light sensitivity of the double layer with dyestuff No. 9 is measured as follows: The half time ( $T_{1/2}$ ) is determined for each wave length range at negative charge by exposure to a xenon lamp, type XBO 150, and placing therebefore monochromatic filters (line filters, half time width 10 to 12 nm, Schott & Gen., Mainz, Germany). By plotting the reciprocal values of the product from half time  $T_{1/2}$  (seconds) and light intensity  $I(\mu\text{W}/\text{cm}^2)$  versus the wave length  $\lambda$  (nm), the spectral light sensitivity of the double layer is obtained which is shown in the attached FIG. 3. The reciprocal value of  $T_{1/2}$ , I means the light energy calculated per unit area which has to be irradiated in order to discharge the layer to half its initial voltage  $U_o$ .

## Example 2

Thioindigo dyestuff layers are provided with a top layer from 1 part by weight of 2-phenyl-4-(2-chlorophenyl)-5(4-diethylaminophenyl)-oxazole (melting point 116° to 117°C) and 1 part by weight of polyester resin, e.g. Dynapol L 206, which are dissolved in tetrahydrofuran and whirl-coated onto the dyestuff layer. After drying for 5 minutes at 120°C, about 10 μm thick layers are obtained.

The photosensitivity is determined as in Example 1 (xenon lamp, 615  $\mu\text{W}/\text{cm}^2$  in the plane of measurement) and compared to that of a zero layer:

| Double layer with dyestuff            | U <sub>o</sub> (V) negative charge | T <sub>1/2</sub> (msec) |
|---------------------------------------|------------------------------------|-------------------------|
| Zero layer                            | 900                                | 500                     |
| Permanent Red Violet MR Formula No. 7 | 600                                | 23                      |
| Indanthren Brilliant Pink 3B          |                                    |                         |

## -Continued

| Double layer with dyestuff                | U <sub>o</sub> (V) negative charge | T <sub>1/2</sub> (msec) |
|-------------------------------------------|------------------------------------|-------------------------|
| Indanthren Brilliant Pink R Formula No. 4 | 800                                | 31                      |

The trisubstituted oxazole derivative is prepared by reacting 4-diethylamino-2'-chloro-benzoin with benzonitrile according to H. Krauch and W. Kunze, "Reaktionen der Organischen Chemie," 3rd edition, 1966, page 335.

## Example 3

Indigo dyestuffs and asymmetrical indigoid dyestuffs yield the following photosensitivities in the double layer arrangement of the invention with a top layer as described in Example 1:

(Measurement in analogy with Example 1; 615  $\mu\text{W}/\text{cm}^2$  in the plane of measurement)

| Double layer with dyestuff | Formula No. | U <sub>o</sub> (V) negative charge | T <sub>1/2</sub> (msec) |
|----------------------------|-------------|------------------------------------|-------------------------|
| Indigo                     | 1           | 1,500                              | 230                     |
| Vat Violet RR              | 11          | 1,100                              | 27                      |
| Algol Violet BBN           | 12          | 1,050                              | 40                      |
| Zero layer                 |             | 800                                | 280                     |

## Example 4

35 Indazin Bordeaux RRL (Formula No. 6 of Cassella Farbwerke Mainkur AG, Frankfurt/Main, Germany), Indanthren Brown RRD (Formula No 15) and Indanthren Printing Brown R (Formula No. 14) of Farbwerke Hoechst AG, Frankfurt/Hochst, Germany, yield the following photosensitivities in vapor deposited dyestuff layers at a top layer according to the Example 1: (Measuring method as in Example 2, 615  $\mu\text{W}/\text{cm}^2$ , xenon lamp)

| Double layer with dyestuff No.     | U <sub>o</sub> (V) negative charge | T <sub>1/2</sub> (msec) |
|------------------------------------|------------------------------------|-------------------------|
| Indazin Bordeaux RRL No. 6         | 850                                | 56                      |
| Indanthren Brown RRD No. 15        | 1,000                              | 100                     |
| Indanthren Printing Brown R No. 14 | 950                                | 115                     |
| Zero layer                         | 800                                | 280                     |

## Example 5

60 For comparison purposes, a dyestuff layer vapor deposited with Indanthren Brilliant Pink 3B (formula 9) and one vapor deposited with Permanent Red Violet MR (Formula 7) are whirl-coated with a solution from polyvinyl carbazole, e.g. Luvican M 170 of BASF, Ludwigshafen, Germany, and 18.6 per cent by weight of an adhesive polyester resin, e.g. Adhesive 49,000 of DuPont, USA, in tetrahydrofuran as the solvent so that

after drying the layer thicknesses of the top layers are 6 and 10  $\mu\text{m}$ , respectively. The photosensitivity is determined as in Example 1; (light intensity 615  $\mu\text{W}/\text{cm}^2$  in the plane of measurement, xenon lamp).

| Double layer with dyestuff No. | top layer thickness ( $\mu\text{m}$ ) | $U_o(\text{V})$ negative charge | $T_{1/2}$ (msec) |
|--------------------------------|---------------------------------------|---------------------------------|------------------|
| 3B / 9                         | 6                                     | 800                             | 280              |
|                                | 10                                    | 800                             | 365              |
| MR / 7                         | 6                                     | 760                             | 410              |
|                                | 10                                    | 875                             | 585              |
| Zero layer                     | 6                                     | 550                             | 1,000            |

### Example 6

The photoconductor material employed in the top layers is 3-bromopyrene resin which has been obtained by condensation of 3-bromopyrene, melting point 94° to 95°C ("Organic synthesis," volume 48 (1968), page 30), with formaldehyde in acetic acid.

To the dyestuffs layers of the following formulae, there is applied a solution from 2 parts by weight of 3-bromopyrene resin and 1 part by weight of polyester resin, e.g. Dynapol L 206. The thickness of the top layer is about 10  $\mu\text{m}$  after drying.

| Double layer with dyestuff                  | $U_o(\text{V})$ negative charge | $T_{1/2}$ (msec) |
|---------------------------------------------|---------------------------------|------------------|
| Indanthren Brilliant Pink 3B, Formula No. 9 | 650                             | 145              |
| Indanthren Brilliant Pink R, Formula No. 4  | 700                             | 215              |
| Permanent Red Violet MR, Formula No. 7      | 675                             | 157              |
| Zero Layer                                  | 650                             | 465              |

### Example 7

To dyestuffs layers from Permanent Red Violet MR (Formula 7) and Indanthren Red Violet RH (Formula 5) there are applied the following binders in a ratio by weight of 1:1 with 2,5-bis-(4-diethylaminophenyl)-oxadiazole-1,3,4 as the photoconductor in tetrahydrofuran as the solvent:

- polycarbonate resin, e.g. Lexan Grade No. 141 of General Electric Comp., USA,
- copolymer from styrene and maleic acid anhydride, e.g. Lytron 820 of Monsanto Comp., USA,
- three-dimensionally cross-linked phenylmethyl siloxane, e.g. silicone resin SR 182, 60 per cent in toluene, of General Electric Comp., USA

The photo-sensitivity of the homogeneous, glossy double layers is determined as in Example 1. (xenon lamp, light intensity 615  $\mu\text{W}/\text{cm}^2$ ):

| Double layer with dyestuff | Binder used in top layer | $U_o(\text{V})$ negative charge | $T_{1/2}$ (msec) |
|----------------------------|--------------------------|---------------------------------|------------------|
| Permanent Red Violet MR    | a                        | 825                             | 29               |

-Continued

| Double layer with dyestuff   | Binder used in top layer | $U_o(\text{V})$ negative charge | $T_{1/2}$ (msec) |
|------------------------------|--------------------------|---------------------------------|------------------|
| Indanthren Red Violet RH     | b                        | 750                             | 25               |
|                              | c                        | 625                             | 16               |
| Indanthren Brilliant Pink 3B | a                        | 925                             | 47               |
|                              | b                        | 875                             | 52               |
|                              | c                        | 800                             | 32               |

### Example 8

Equivalent quantities of a polyester containing hydroxyl groups, e.g. Desmophen 1100 (2g), and of a polyfunctional isocyanate, e.g. Desmodur HL (3 g), are applied together with 2,5-bis-(4-diethylaminophenyl)-oxadiazole-1,3,4 in tetrahydrofuran to dyestuff layers from Permanent Red Violet MR (Formula 7) and Indanthren Brilliant Pink 3B (Formula 9) in a thickness of about 10  $\mu\text{m}$ . After drying and hardening for about 5 to 15 minutes at 120°C, glossy, homogeneous top layers are obtained.

The photosensitivity is determined as in Example 1 (xenon lamp, light intensity 615  $\mu\text{W}/\text{cm}^2$ ):

| Dyestuff                     | $U_o(\text{V})$ negative charge | $T_{1/2}$ (msec) | $\Delta U_o$ |
|------------------------------|---------------------------------|------------------|--------------|
| Permanent Red Violet MR      | 650                             | 19               | 120          |
| Indanthren Brilliant Pink 3B | 835                             | 20               | 90           |

### Example 9

A 2 per cent solution from a polyamide resin, e.g. Elvamide 8061 of Du Pont, USA, in trichloroethylene-methanol (1:1) is coated on a polyester film (100  $\mu\text{m}$ ) vapor-deposited with aluminum. The thickness of the top layer is below 1  $\mu\text{m}$  since the layer weight is 0.2 g/m<sup>2</sup>.

To this organic intermediate layer, there are vapor-deposited various dyestuffs, such as Indazin Bordeaux RRL (Formula 6) or Vat Violet RR (Formula 11) in analogy with Example 1. To this layer, there is applied a top layer as described in Example 1; after drying, the layer thickness is about 9 to 10  $\mu\text{m}$ .

The photosensitivity is measured according to the method indicated in Example 1 (light intensity about 615  $\mu\text{W}/\text{cm}^2$ , xenon lamp).

| Double layer with dyestuff | $U_o(\text{V})$ negative charge | $T_{1/2}$ (msec) | $\Delta U_o$ |
|----------------------------|---------------------------------|------------------|--------------|
| Indazin Bordeaux RRL       | 1,175                           | 155              | 45           |
| Vat Violet RR              | 1,150                           | 280              | 25           |
| Zero layer                 | 1,020                           | 370              | —            |

### Example 10

Dyestuff layers from Indanthren Printing Violet BBF (Formula 13) are coated with solutions from a. 1 part by weight of 2,5-bis-(4-diethylaminophenyl)-oxadiazole-1,3,4 and 1 part by weight of

- polyester resin, e.g. Dynapol L 206 of Dynamit Nobel AG, Troisdorf, Germany,  
 b. same as a) plus  $10^{-3}$  part by weight of Brilliant Green  
 c. same as a) plus 0.1 part by weight of 3,5-dinitrobenzoic acid.

The thicknesses of the top layers are about 10  $\mu\text{m}$ .

The following photosensitivities are determined: (measuring method as in Example 1, xenon lamp, light intensity: 615  $\mu\text{W}/\text{cm}^2$ ).

| Double layers | $U_o(\text{V})$<br>negative<br>charge | $T_{1/2}$<br>(msec) |
|---------------|---------------------------------------|---------------------|
| a             | 900                                   | 38                  |
| b             | 975                                   | 48                  |
| c             | 1,050                                 | 75                  |

### Example 11

Homogeneous dyestuff layers are obtained within 1 minute with the dyestuffs Brilliant Indigo B and Brilliant Indigo 4B (Formulae 16 and 17) by vapor-deposition onto a aluminum foil (100  $\mu\text{m}$ ) at 200° and 270°C under a reduced pressure of  $10^{-3}$  to  $10^{-4}$  mm Hg.

These layers are coated with a solution as described in Example 1. After drying, the layer thicknesses are about 10  $\mu\text{m}$ .

The photosensitivity is determined as in Example 1 (xenon lamp, light intensity: 487  $\mu\text{W}/\text{cm}^2$ ):

| Double layer<br>with dyestuff | $U_o(\text{V})$<br>negative<br>charge | $T_{1/2}$<br>(msec) |
|-------------------------------|---------------------------------------|---------------------|
| Brilliant Indigo B            | 1,050                                 | 92                  |
| Brilliant Indigo 4B           | 1,150                                 | 39                  |

It will be obvious to those skilled in the art that many modifications may be made within the scope of the present invention without departing from the spirit thereof, and the invention includes all such modifications.

What is claimed is:

1. An electrophotographic recording material consisting of an electro-conductive support material and a photoconductive double layer of organic materials which consists of a homogeneous, opaque, charge-carrier producing dyestuff layer from a compound of the general formula



in which  $X_1$  and  $X_2$  are identical or different and stand for  $-\text{NH}-$  or  $-\text{S}-$  and  $\text{Ar}$  and  $\text{Ar}'$  may be substi-

tuted, such compounds being particularly suitable as are substituted in peri position to the  $=\text{C}=\text{O}$ ,  $-\text{S}-$  or  $-\text{NH}-$  group in the five-membered ring, and of a transparent top layer of insulating materials with at least one charge transporting compound, in which the transparent top layer consists of a charge transporting, monomeric, heterocyclic compound substituted by at least one dialkyl amino group or two alkoxy groups and having an extended  $\pi$ -electron system or of a condensation product from 3-bromopyrene and formaldehyde and of a binder.

2. A material according to claim 1, in which the heterocyclic compound is selected from the group of oxazoles, oxadiazoles, triazoles, imidazoles, and pyrazoles.

3. A material according to claim 1, in which the heterocyclic compound is an oxadiazole.

4. A material according to claim 1, in which the heterocyclic compound is 2,5-bis-(4-diethylaminophenyl)-oxadiazole-1,3,4.

5. A material according to claim 1, in which the heterocyclic compound is an oxazole.

6. A material according to claim 1, in which the heterocyclic compound is 2-phenyl-4-(2-chlorophenyl)-5-(4-diethylaminophenyl)-oxazole.

7. A material according to claim 1, in which the dyestuff layer has a thickness from about 0.005 to about 2  $\mu\text{m}$  and the transparent top layer a thickness from about 5 to 20  $\mu\text{m}$ .

8. A material according to claim 1, in which the transparent top layer consists of a mixture of the charge transporting compound and the binder in a ratio by weight of about 1:1.

9. A material according to claim 1, in which the binder is selected from the group of polyesters, copolymers, silicone resins, reactive resins from polyethers or polyesters and polyfunctional isocyanates, of copolymers of styrene with maleic acid anhydride, and of polycarbonates.

10. A material according to claim 1, in which the binder is a copolymer from iso- and terephthalic acid and a glycol.

11. A material according to claim 1, in which the binder is a copolymer from styrene and maleic acid anhydride.

12. A material according to claim 1, in which the binder is a reactive resin from polyethers or polyesters and polyfunctional isocyanates.

13. A material according to claim 1, in which the binder is a silicone resin from three-dimensionally cross-linked phenyl methyl siloxane.

14. A material according to claim 1, in which the binder is a polycarbonate resin.

15. A material according to claim 1, in which the transparent top layer additionally contains sensitizers and/or substances forming charge transfer complexes.

16. A material according to claim 1, in which the photoconductive double layer is above an insulating intermediate layer on the support material.

\* \* \* \* \*